# EUROPEAN PATENT SPECIFICATION

(11) **EP 3 406 750 B1**
(45) Date of publication and mention of the grant of the patent: **05.04.2023**
(21) Application number: 18173837.8
(22) Date of filing: 23.05.2018
(51) Int. Cl.: C22F 1/04

(54) **SINGLE-PIECE EXTENDED LAMINAR FLOW INLET LIPSKIN**
EINSTÜCKIG VERLÄNGERTE RINGLIPPE(LIPSKIN) MIT LAMINAREM FLUSS
PIÈCE EN ALUMINIUM AÉROSPATIAL (LIPSKIN)

(30) Priority: 24.05.2017 US 201715603899; 21.06.2017 NL 1042437
(43) Date of publication of application: 28.11.2018
(73) Proprietor: The Boeing Company, Arlington, VA 22202 (US)
(72) Inventor: LEON, Luis, Chicago, IL 60606-1596 (US); NILL, Michael, Chicago, IL 60606-1596 (US); SAHA, Pradip K., Chicago, IL 60606-1596 (US); OLIVER, Carol S., Chicago, IL 60606-1596 (US); JOHNSON, Ricole A., Chicago, IL 60606-1596 (US)
(74) Representative: Duxbury, Stephen

(56) References cited:
- US-B1- 8 323 427
- US-B2- 9 090 950
- YUAN S J ET AL: "Formability and microstructural stability of friction stir welded Al alloy tube during subsequent spinning and post weld heat treatment", MATERIALS SCIENCE AND ENGINEERING: A, vol. 558, 19 August 2012 (2012-08-19), pages 586-591, XP028938841, ISSN: 0921-5093, DOI: 10.1016/J.MSEA.2012.08.056
- N.N.: "Custom Machines Create Engine Lip Skins on Boeing Aircraft", , 1 December 2016 (2016-12-01), XP055487595, Retrieved from the Internet: URL:https://www.techbriefs.com/component/c ontent/article/tb/features/application-bri efs/26069 [retrieved on 2018-06-25]
- Saha Pradip K.: "Chapter 8: Cold Forming of Flat Sheet" In: "Aerospace Manufacturing Processes", 19 September 2016 (2016-09-19), CRC Press, US, XP055798890, ISBN: 978-1-4987-5605-1 pages 205-252, DOI: 10.1201/9781315367965, Retrieved from the Internet: URL:https://ebookcentral.proquest.com/lib/ epo-ebooks/reader.action?docID=4694245&ppg =296>
- Anonymous: "Review of Explosive (chemical) Forming", DDC Report, 1 April 1965 (1965-04-01), page 80, XP055798906,
- Sanders Daniel ET AL: "Superplastically Formed Friction Stir Welded Tailored Aluminum and Titanium Blanks for Aerospace Applications", 6th EUROSPF Conference, 1 September 2008 (2008-09-01), pages 1-9, XP055798891,
- Strohecker D.E. ET AL: "EXPLOSIVE FORMING OF METALS", DMIC Report 203, 8 May 1964 (1964-05-08), page 11, XP055798898,
- Ghizdavu Victor ET AL: "Explosive forming - economical technology for aerospace structures", INCAS BULLETIN, vol. 2, no. 4, 1 January 2010 (2010-01-01) , pages 107-117, XP055798903, Bucharest ISSN: 2247-4528, DOI: 10.13111/2066-8201.2010.2.4.15

## Description

The present invention relates generally to the field of fabricating metal structures. More specifically, the present invention relates to manufacturing a metal structure or component comprising shaping the metal structure or component while in specified heat-treatment conditions, and introducing a friction stir weld into the metal structure or component with the friction stir weld being maintained in the finished component. The present disclosure further relates to the manufacture of components and assemblies used to make lipskins for aircraft engine nacelles.

Laminar flow is the smooth, uninterrupted flow of air over the contour of wings, fuselages, or other parts of an aircraft in flight. Laminar flow is most often found at the front of a streamlined body. If the smooth flow of air is interrupted, turbulence is created, which can result in drag acting on the body. Increases in deviation away from optimal laminar flow at aircraft surfaces can result in an increase in fuel consumption, and therefore a commensurate increase in cost of operation.

Many known aircraft engines, for example jet engines and turbofan jet engines are surrounded by an annular, barrel-shaped nacelle. At least some known nacelles include a lipskin at the leading edge, or inlet, of the nacelle. While some large structures have been formed in a unitary fashion to reduce transverse weld lines or other couplings that could impact laminar flow, such unitary forming processes (e.g. spin-forming, etc.) are time-consuming, expensive and difficult or impractical in terms of size limitations for producing spin-formed lipskins of a desired, large size. Further, spin-formed lipskins may exhibit undesirable waves or ripples that could adversely affect laminar flow, leading to undesirable turbulence, increased fuel consumption, and/or increased cost of operation.

In attempts to solve the potential restrictiveness of spin-forming or other processes, some known methods for lipskin construction for aircraft engine nacelles have included the introduction of friction stir welds during lipskin construction, followed by removal of the welds during shaping, finishing, and other manufacturing processes, and further followed by the introduction of additional coupling components and parts (e.g. doublers). However, additional processing steps are often time-consuming, and the addition of parts in an aircraft assembly is often undesirable due to the commensurate increase in weight, assembly complexity, manufacturing time, additional inspections, etc., all of which can increase the overall cost of operating and maintaining the aircraft.

The abstract of the document from Yuan S J Et al 'Formability and microstructural stability of friction stir welded Al alloy tube during subsequent spinning and post weld heat treatment', Materials Science and Engineering: A Volume 558, 15 December 2012, Pages 586-591,XP028938841, ISSN: 0921-5093, DOI:10.10.1016/J.MSEA.2012.08.056, reads: "Subsequent spinning combined with post weld heat treatment (PWHT) was imposed to the friction-stir welding tube, and the effects of PWHT on the formability and microstructural stability of the FSW tubes were investigated in detail. The formability of tubes, evaluated by the hydraulic bulge test, is significantly improved after spinning and PWHT due to the grain refinement, removal of the thickness reduction and heterogeneous microstructure of the weld. Even abnormal grain growth occurs, the tubes still show a relatively high formability compared to the extruded tubes. The PWHT process plays key roles in controlling the size of precipitates and subgrains, and consequently dominates the microstructure stability that is correlated to the strain hardenability and formability of the tubes."

The abstract of US 9,090,950 B2 reads: "The present invention provides a process for suppressing abnormal grain growth in friction stir welded aluminum alloys by inserting an intermediate annealing treatment ("IAT") after the welding step on the article. The IAT may be followed by a solution heat treatment (SHT) on the article under effectively high solution heat treatment conditions. In at least some embodiments, a deformation step is conducted on the article under effective spin-forming deformation conditions or under effective superplastic deformation conditions. The invention further provides a welded article having suppressed abnormal grain growth, prepared by the process above. Preferably the article is characterized with greater than about 90% reduction in area fraction abnormal grain growth in any friction-stir welded nugget."

Aspects of the present disclosure of the present invention are directed to methods for forming metal lipskins for engine nacelles and the lipskins and nacelles so formed, as well as structures comprising the nacelles that comprise the lipskins, where the introduction of at least one "fly-away" weld (including without limitation, one friction stir weld), and forming processes of a metal lipskin occurs in specified conditions of the metal such that the "fly-away" weld is maintained in the finished lipskin.

An aspect of the present disclosure of the invention is directed to a method for making a heat-treated structure formed of metal, the method comprising performing a first heat-treating process on a roughly-shaped metal workpiece in an annealed condition to transition the roughly-shaped metal workpiece from the annealed condition into a first hardened condition, the roughly-shaped metal workpiece in the annealed condition comprising at least one friction stir weld; forming the roughly-shaped metal workpiece into a shaped metal workpiece while the roughly-shaped metal workpiece is in the first hardened condition, the shaped metal workpiece comprising one of a near-finally-shaped metal workpiece or a finally-shaped metal workpiece; and performing a second heat-treating process on the shaped workpiece to transition the shaped metal workpiece from the first hardened condition to a second hardened condition, wherein the forming process is selected from the group consisting of: a super-plastic forming process; a super-plastic/diffusion bond forming process; an explosion forming process; and combinations thereof, wherein performing the first heat-treating process comprises performing a T4 heat-treating process on the roughly-shaped metal workpiece, wherein the metal is a 2000-, 4000-, 6000-, or 7000-series aluminum alloy.

The method preferably comprises forming the second hardened metal workpiece into a shaped metal workpiece, said shaped metal workpiece being in one of a near-finally-shaped metal workpiece or a finally-shaped metal workpiece.

The shaped metal workpiece can be, or may comprise, a near-finally-shaped metal workpiece, the method preferably further comprising forming the near-finally-shaped metal workpiece into the finally-shaped metal workpiece while the near-finally-shaped metal workpiece is in the second hardened condition.

The shaped metal workpiece may comprise a finally-shaped metal workpiece, the method preferably further comprising using one or more forming processes to shape the roughly-shaped metal workpiece into the finally-shaped metal workpiece.

Before the step of performing the first heat-treating process on the roughly-shaped metal workpiece, a metal sheet can be formed into the roughly-shaped metal workpiece while the metal sheet is in the annealed condition, preferably wherein the step of forming a metal sheet comprises rolling the metal sheet into the roughly-shaped metal workpiece.

The metal sheet is preferably in an annealed condition, and is formed into the roughly-shaped metal workpiece by a process selected from the group consisting of: a super-plastic forming process; a super-plastic/diffusion bond forming process; a form-die forming process; an explosion forming process; and combinations thereof.

The roughly-shaped workpiece can be a conical-shaped metal workpiece or a frusto-conical-shaped metal workpiece.

Performing the second heat-treating process may further comprise:
performing at least one age-hardening process on the roughly-shaped metal workpiece in the first and/or second hardened condition.

The age-hardening process can be a natural aging process when the roughly-shaped metal is in the first hardened condition.

The age-hardening process can be an artificial aging process when the roughly shaped metal is in the second hardened condition

The second hardened condition may comprise a second age-hardened condition.

The step of performing the second heat-treating process can further comprise solution heat-treating the metal.

Performing the second heat-treating process may comprise performing a T-6 heat-treating process.

Having thus described variations of the invention in general terms, reference will now be made to the accompanying drawings, which are not necessarily drawn to scale, illustrating examples according to aspects of the present disclosure, wherein:
- figure 1 is a flowchart illustrating an exemplary forming method of the present disclosure;
- figure 2 is a flowchart illustrating an exemplary method of the present disclosure;
- figure 3 is a flowchart illustrating an exemplary method of the present disclosure;
- figure 4 is a flowchart illustrating an exemplary method of the present disclosure;
- figure 5 is a flowchart illustrating an exemplary method of the present disclosure;
- figure 6 is a flowchart illustrating an exemplary method of the present disclosure;
- figure 7 is a flowchart illustrating an exemplary method of the present disclosure;
- figures 8A, 8B, and 8C are cross-sectional side-views of a workpiece progressing through stages of a forming process from a rough-shaped metal workpiece into a shaped, near-finally shaped and finally-shaped metal workpiece, according to aspects of the present disclosure;
- figure 9 is a perspective view of a roughly-shaped metal workpiece in a frusto-conical orientation;
- figure 10 is a perspective view of a roughly-shaped metal workpiece being oriented into a forming block of a forming process, according to aspects of the present disclosure;
- figures 11A, 11B, 11C, 11D, and 11E are cross sectional side views of forming blocks in a forming process used to transform a roughly-shaped metal workpiece into a near-finally-shaped and finally-shaped metal workpiece;
- figure 12 is a perspective view of a final-shaped metal workpiece as lipskin for an nacelle made according to aspects of the present disclosure; and
- figure 13 is a perspective view of an aircraft comprising an engine nacelle.

Methods for constructing unitary, or single-piece, aircraft engine lipskins that can provide improved laminar flow are disclosed herein. The methods and apparatuses disclosed herein provide a lightweight, efficient, reproducible and high-performance engine nacelle lipskin made from a heat-treatable metal that has been shaped and tempered according to specified protocols that facilitate unitary formation of a large contoured metal structure without requiring introduction of additional components to structurally reinforce areas of the unitary structure where welds occur. That is, in the structures and methods according to aspects of the present application, the welds made in the structures are retained in the finished structure.

Retention of the welds in structures used in aircraft (e.g. lipskins on aircraft nacelle assemblies) allows such welds to be so-called "fly-away" welds that are retained in the finished structure. Without being bound to any particular theory, the shaping of the metals used to make the lipskins, according to aspects of the present disclosure, is predominantly conducted and accomplished while the metal is in the annealed condition. The order of shaping in the annealed condition can allow for weld retention in a finished product due to internal metal stresses being managed in a predetermined way that obviates the need to remove such welds and introduce additional reinforcing components that would complicate the manufacturing process and add weight to a structure comprising the lipskin.

For the purposes of the present disclosure, "heat-treatable metals" refer to heat-treatable metals that include aluminum and the 2000-, 4000-, 6000-, and 7000-series aluminum alloys.

According to aspects of the present disclosure, a metal workpiece in the annealed state can be formed into a roughly-shaped metal workpiece by being subjected to at least one forming process. For the purpose of the present disclosure, super-plastic processes, super-plastic/diffusion bond processes, form-die processes, and explosive-forming processes are examples of a forming process and may be equivalently and interchangeably referred to as "forming processes".

Explosive-forming processes may be equivalently and interchangeably referred to as "explosion-molding", "explosive molding", "explosion-forming" or "high-energy hydroforming" (HEHF) processes. An explosive-forming process is a metalworking process where an explosive charge is used to supply the compressive force (e.g. a shockwave) to a metal workpiece against a form (e.g. a mold) otherwise referred to as a "die". Explosive-forming is typically conducted on materials and structures of a size too large for forming such structures using a punch or press to accomplish the required compressive force. According to one explosive-forming approach, a metal workpiece, up to several inches thick, is placed over or proximate to a die, with the intervening space, or cavity, optionally evacuated by a vacuum pump. The entire apparatus is submerged into an underwater basin or tank, with a charge having a predetermined force potential detonated at a predetermined distance from the metal workpiece to generate a predetermined shockwave in the water. The water then exerts a predetermined dynamic pressure on the workpiece against the die at a rate on the order of milliseconds. The die can be made from any material of suitable strength to withstand the force of the detonated charge such as, for example, concrete, ductile iron, etc. The tooling should have higher yield strength than the metal workpiece being formed.

Explosive forming processes are sometimes divided into two groups, depending upon the position of the explosive charge relative to the workpiece. According to the "stand off" method, a workpiece is placed over a die with the intervening space evacuated by a vacuum, with the entire assembly immersed under water, preferably in a basin or tank. The explosive material is then placed at a predetermined distance from the assembly and detonated. According to the "contact method", an explosive charge is placed in direct contact with the workpiece and the detonation produces interface pressures on the workpiece surface up to several million pounds per square inch (psi).

Superplastic forming is a forming process that typically uses high temperature and gas pressure to form particular materials onto a single step mold. Superplastic forming can create very detailed metal parts including aluminum and titanium. Superplasticity is the ability of a material to experience extremely high elongations on the order of 200% or more. For a material to elicit superplastic behavior, there are typical criteria including, for example, an extremely fine grain size (a few micrometers or less), with generally uniform and equiaxed grain structure; high temperatures (usually on the order of half the melting temperature); low strain rates (e.g. on order of 10⁻²/seconds or lower).

Friction stir welding (FSW) refers to a process for the solid-state joining of two workpieces using a non-consumable tool without melting the material of the workpiece(s). Heat is generated by friction between a rotating tool and the workpiece, resulting in a softened region proximate to the FSW tool. As the FSW tool proceeds along a desired joining line, the tool mechanically intermixes the material of the workpieces to be joined. In this way, hot and softened metal of the workpieces is forged by the mechanical pressure that is applied by the FSW tool, resulting in a solid state deformation of dynamic recrystallization of the workpiece materials without melting the workpieces. While aspects of the present disclosure describe producing and retaining friction stir welds in the metals used, the present disclosure contemplates, without limitation, any type of welds can be "fly-away welds". As explained above, "fly-away welds" refer to welds in components and parts that remain in the part or component as used in flight. In other words, "fly-away welds" are retained in the finished structures as opposed to being removed from the structures before use.

According to the present disclosure, a heat-treated structure is a structure, preferably a metal structure, that is exposed to heat-treating. Heat-treating for metals (especially metal alloys) manipulates the properties of the metal by controlling rates of diffusion and the rate of cooling within a metal's microstructure. Heat-treating predictably alters the mechanical properties of a metal, manipulating properties including hardness, strength, ductility, elasticity, etc. The present specification discloses first heat-treating processes and second heat-treating processes to achieve metal workpieces having a particular "state" or heat-treatment "condition". According to the present disclosure, for aluminum alloys, the heat-treatment conditions include an annealed condition, a first hardened condition, and a second hardened condition.

For aluminum alloys, the annealed condition is used to describe alloys used for sheet workpieces made by some shaping processes. The annealed condition is the lowest strength condition for a metal alloy workpiece. Annealing is a heat treatment that alters the physical properties of a material to increase ductility and reduce hardness, making the material more "workable". In annealing, atoms migrate in a material's crystalline lattice, with the number of dislocations decreasing, leading to a change in ductility and hardness. A dislocation refers to the primarily linear defects present throughout a material's crystalline structure and the internal stresses caused thereby. Annealing conditions for aluminum alloys vary according to individual aluminum alloys, but generally require exposing the aluminum alloy to a temperature of from about 650°F (343.3°C) to about 770°F (410°C) for 2 to 3 hours, followed by slow cooling to about 500°F (260°C) followed by uncontrolled cooling rates to room temperature. Specific temperatures, times, cooling rates, etc. can differ from the examples above, depending upon which metal (e.g. aluminum alloy) is being treated.

The "T" temper designation for heat-treated (e.g. heat-treatable) aluminum and aluminum alloys includes a number that indicates a basic type of treatment. Of particular interest for the present disclosure are the T4 and T6 conditions. As used herein, the T4 condition is an example of a "first hardened condition". A T4 condition indicates that the T4 treated alloy has incurred a solution heat treatment and, has naturally aged to a stable condition. As used herein, the T6 condition is an example of a "second hardened condition". A T6 condition indicates that the T6 treated alloy has been solution heat treated and, without any significant cold working, has been artificially aged to achieve additional precipitation hardening to become stable metalurgically.

According to an aspect of the present disclosure, an aluminum alloy may be provided in the annealed condition as a sheet of material (i.e., the "O" condition) with either partial or full anneal cycles intermittently conducted on the aluminum alloy. The annealed aluminum alloy is brought to the first hardened condition, such as the T4 condition, via a solution heat treatment, and bringing the aluminum alloy sheet to a temperature above 900°F (482.2°C) for a time that is dependent on the particular alloy and the thickness of the sheet) followed by quenching in water or glycol. The aluminum alloys selected are precipitation age-hardenable, allowing the alloys to naturally age at room temperature. If desired, the aging in the T4 condition may be tailored by placing the alloy in the T4 condition in dry ice or in a freezer. The alloy sheet in the first hardened condition (e.g., the T4 condition) may then be formed into a roughly-shaped metal workpiece that includes introducing at least one friction stir weld introduced in the annealed condition to shape the metal workpiece as desired. According to a contemplated aspect, in the case of forming lipskins for aircraft engine nacelles, the alloy in the annealed condition is shaped and friction stir welded to a roughly-shaped metal workpiece, and then the alloy in the first hardened condition is shaped or to a near-finally-shaped metal workpiece or finally-shaped workpiece.

According to aspects of the present disclosure, during the first-hardened process, the alloy is subjected to at least one forming process that includes, for example, an explosive forming process, to create the near-finally-shaped metal workpiece or the finally-shaped metal workpiece. According to contemplated aspects, most of the forming of the aluminum alloy into the near-finally-shaped metal workpiece is conducted with the alloy in the first hardened condition (e.g., the T4 condition). The near-finally-shaped metal workpiece is then brought to a second hardened condition (i.e. T6 condition) by artificially aging the metal workpiece. For example, for aluminum alloy Al-2219, the cycle time and temperature is 375°F (190.5°C) for 36 hours.

Figures 1-7 are flowcharts describing aspects of the present disclosure. Consistent with particular aspects of the present disclosure, figure 1 is directed to a method 10 for making a heat-treated structure formed of metal. The method 10 includes forming 12 a metal sheet into a roughly-shaped metal workpiece having a friction stir weld while the metal sheet is in an annealed condition. One example of the roughly-shaped metal workpiece is the metal workpiece 90 having at least one friction stir weld 92 as shown in figure 9, which is described in more detail below.

Method 10 includes step 12 performed in a manner consistent with aspects of the present disclosure using forming processes such as rolling or other physical shaping means suitable to physically transform and shape a metal from a first, or initial, orientation to a subsequent orientation. Further forming processes to transform metal to a roughly-shaped metal workpiece, as contemplated by aspects of the present disclosure, may take place in step 12 including subjecting the metal sheet to super-plastic processes, super-plastic/diffusion bond processes, form-die processes, explosive-forming processes, and combinations thereof. The roughly-shaped state of the metal workpiece, according to aspects of the present disclosure, therefore contemplates the state of the metal work-piece between the initial form of a metal (e.g., a metal sheet that may be substantially planar) and a shaped (i.e., near-finally-shaped or finally-shaped) metal workpiece that has been subjected to subsequent forming processes after attaining the roughly-shaped metal workpiece.

The method 10 further includes performing 14 a first heating-treating process on the roughly-shaped metal workpiece to transition the roughly-shaped metal workpiece from an annealed condition to a first hardened condition. The roughly-shaped metal workpiece includes the at least one friction stir weld (e.g., friction stir weld 92 shown in figure 9). When the metal workpiece is aluminum or an aluminum alloy, the first hardened condition is the T4 condition. The method 10 includes forming 16 the roughly-shaped metal workpiece into a shaped metal workpiece while the roughly-shaped metal workpiece is in the first hardened condition. An example of the shaped metal workpiece is the metal workpiece 114b, 114c, 114d, 114e, and 120 as shown in figure 9 and figures 11B, 11C, 11D, 11E, and FIG 12, which is described in more detail below. According to aspects of the present disclosure, the shaped metal workpiece retain and includes the friction stir weld 92 introduced to the roughly-shaped metal workpiece as shown in figure 9. The shaped metal workpiece comprises one of a near-finally-shaped metal workpiece or a finally-shaped metal workpiece.

According to aspects of the present disclosure, method 10 includes forming 16 processes used to transform a roughly-shaped metal workpiece into the shaped (i.e., near-finally-shaped or finally-shaped) metal workpieces include subjecting the metal sheet to super-plastic processes, super-plastic/diffusion bond processes, form-die processes, explosive-forming processes, and combinations thereof. When an explosive-forming process is used in step 16, the explosive-forming process also includes the quenching step of the first heat-treating process.

Aspects of the method 10 include performing 18 a second heat-treating process on the shaped workpiece to transition the shaped metal workpiece from the first hardened condition to produce a second hardened condition. When the metal workpiece is aluminum or an aluminum alloy, the second hardened condition is a T6 condition. At least one forming process can be performed while the metal is in the second hardened condition. However, all of the forming processes on the roughly-shaped workpiece (e.g., forming the roughly-shaped metal workpiece into the shaped metal workpiece) may be completed while the metal is in the first hardened condition.

Consistent with particular aspects of the present disclosure, figure 2 is directed to a method 20 for making a heat-treated structure formed of metal. The method described in figure 2 is similar to the method outlined in figure 1, except the method 20 contemplates starting with a roughly-shaped metal workpiece rather than, for example, a flat sheet of metal. The method 20 includes performing 22 a first heat-treating process on a roughly-shaped metal workpiece in an annealed condition to transition the roughly-shaped metal workpiece from an annealed condition to a first hardened condition, with the roughly-shaped metal workpiece comprising at least one friction stir weld introduced to the metal workpiece in the annealed condition. One example of the roughly-shaped metal workpiece is the metal workpiece 90 having at least one friction stir weld 92 as shown in figure 9, which is described in more detail below. The first hardened condition of the metal is in the T4 condition when the metal workpiece is aluminum or an aluminum alloy.

The method 20 further includes forming 24 the roughly-shaped metal workpiece into a shaped metal workpiece while the roughly-shaped metal workpiece is in the first hardened condition, with the shaped metal workpiece being one of a near-finally-shaped metal workpiece or a finally-shaped metal workpiece. According to aspects of the present disclosure, the forming process(es) 24 used to transform a roughly-shaped metal workpiece into the shaped (i.e., near-finally-shaped or finally-shaped) metal workpiece includes subjecting the roughly-shaped metal workpiece to at least one forming process that includes super-plastic processes, super-plastic/diffusion bond processes, form-die processes, explosive-forming processes, and combinations thereof. An example of the shaped metal workpiece is the metal workpiece 114b, 114c, 114d, 114e, and 120, as shown in figures. 11B, 11C, 11D, 11E, and FIG 12, and which is described in more detail below. According to aspects of the present disclosure, the shaped metal workpiece retains and includes the friction stir weld 92 introduced to the roughly-shaped metal workpiece as shown in figure 9. When an explosive-forming process is used in step 24, the explosive-forming process also includes the quenching step of the first heat-treating process.

The method 20 further includes performing 26 a second heat-treating process on the shaped workpiece to transition the shaped metal workpiece from the first hardened condition to produce a second hardened condition. When the metal workpiece is aluminum or an aluminum alloy, the second hardened condition is the T6 condition. At least one forming process can be performed while the metal is in the second hardened condition. However, as contemplated by method 20, all of the forming processes on the roughly shaped metal workpiece (e.g., forming the roughly-shaped metal workpiece into the shaped metal workpiece) may be completed while the metal is in the first hardened condition.

Consistent with particular aspects of the present disclosure, figure 3 is directed to a method 30 for making a heat-treated structure formed of metal. Whereas FIGs 1 and 2 outline methods, 10 and 20 respectively, where the roughly-shaped metal workpiece is formed into a shaped metal workpiece in the first hardened condition, as shown in figure 3, a method 30 is further defined such that at least some forming of the metal workpiece into the shaped metal workpiece occurs after the metal workpiece is in the second hardened condition. The method 30 includes performing 32 a first heat-treating process on a roughly-shaped metal workpiece in an annealed condition (with the workpiece in an annealed condition including at least one friction stir weld) to transition the roughly-shaped metal workpiece into a first hardened condition to produce a first-hardened metal workpiece. One example of the roughly-shaped metal workpiece is the metal workpiece 90 having at least one friction stir weld 92 as shown in figure 9, which is described in more detail below. The first hardened condition of the metal is the T4 condition when the metal workpiece is aluminum or an aluminum alloy.

The method 30 further includes performing 34 a second heat-treating process on the first-hardened metal workpiece to transition the first-hardened workpiece a second hardened condition to produce a second-hardened metal workpiece. When the metal workpiece is aluminum or an aluminum alloy, the second hardened condition is the T6 condition.

The method 30 further includes forming 36 the second-hardened metal workpiece into a shaped metal workpiece, with the shaped metal workpiece being in one of a near-finally-shaped metal workpiece or a finally-shaped workpiece. An example of the shaped metal workpiece is the metal workpiece 114b, 114c, 114d, 114e, and 120 as shown in figures. 11B, 11C, 11D, 11E, and FIG 12, which is described in more detail below. According to aspects of the present disclosure, the shaped metal workpiece retains and includes the friction stir weld 92 introduced to the roughly-shaped metal workpiece as shown in figure 9. According to aspects of the present disclosure, in method 30, forming processes 36 used to transform a roughly-shaped metal workpiece into the shaped (i.e. near-finally-shaped or finally-shaped) metal workpiece includes subjecting the metal workpiece to super-plastic processes, super-plastic/diffusion bond processes, form-die processes, explosive-forming processes, and combinations thereof. As contemplated by method 30, all of the forming processes on the roughly shaped metal workpiece (e.g. forming the roughly-shaped metal workpiece into the shaped metal workpiece) may be completed while the metal is in the second hardened condition.

Consistent with particular aspects of the present disclosure, figure 4 is directed to a method 40 for making a heat-treated structure formed of metal. Whereas figuress 1 and 2 outline methods, 10 and 20 respectively, where the roughly-shaped metal workpiece is formed into a shaped metal workpiece in the first hardened condition, as shown in figure 4, a method 40 is further defined such that at least some forming of the metal workpiece into the shaped metal workpiece occurs after the metal workpiece is in the second hardened condition. Further, as compared with the method 30 outlined in figure 3, in figure 4 the metal workpiece is formed into a near-finally-shaped and finally-shaped metal workpiece while the metal workpiece is in the second hardened condition. The method 40 includes performing 32 a first heat-treating process on a roughly-shaped metal workpiece (with the workpiece in an annealed condition including at least one friction stir weld) to transition the roughly-shaped metal workpiece into a first hardened condition to produce a first-hardened metal workpiece. One example of the roughly-shaped metal workpiece is the metal workpiece 90 having at least one friction stir weld 92 as shown in figure 9, which is described in more detail below. The first hardened condition of the metal is the T4 condition when the metal workpiece is aluminum or an aluminum alloy.

The method 40 further includes performing 34 a second heat-treating process on the first-hardened metal workpiece to transition the first-hardened workpiece to a second hardened condition to produce a second-hardened metal workpiece. When the metal workpiece is aluminum or an aluminum alloy, the second hardened condition is the T6 condition.

The method 40 further includes forming 37 the second-hardened metal workpiece into a near-finally-shaped metal workpiece. An example of a near-finally-shaped metal workpiece is the metal workpiece 114d as shown in figure 11D, which is described in more detail below. According to aspects of the present disclosure, the shaped metal workpiece retains and includes the friction stir weld 92 introduced to the roughly-shaped metal workpiece as shown in figure 9. According to aspects of the present disclosure, the method 40, in step 37 the forming processes used to transform a roughly-shaped metal workpiece into the near-finally-shaped metal workpiece includes subjecting the metal sheet to super-plastic processes, super-plastic/diffusion bond processes, form-die processes, explosive-forming processes, and combinations thereof.

The method 40 further includes forming 42 the near-finally shaped metal workpiece into the finally-shaped metal workpiece while the near-finally-shaped metal workpiece is in the second hardened condition. According to aspects of the present disclosure, the method 40, forming processes 42 used to transform a roughly-shaped metal workpiece into the shaped (i.e. near-finally-shaped or finally-shaped) metal workpiece including subjecting the metal sheet to super-plastic processes, super-plastic/diffusion bond processes, form-die processes, explosive-forming processes, and combinations thereof. An example of the finally-shaped metal workpiece is the metal workpiece 114e and 120 as shown in figure 11E and figure 12, which is described in more detail below. As contemplated by method 40, all of the forming processes on the roughly shaped metal workpiece (e.g., forming the roughly-shaped metal workpiece into the near-finally-shaped metal workpiece and the finally-shaped metal workpiece) may be completed while the metal is in the second hardened condition

Consistent with particular aspects of the present disclosure, figure 5 is directed to a method 50 for making a heat-treated structure formed of metal. Figures 1 and 2 outline methods, 10 and 20 respectively, where the roughly-shaped metal workpiece is formed into a shaped metal workpiece in the first hardened condition. Further, as compared with the method 30 outlined in figure 3, in figure 4 (method 30) and figure 5 (method 50) the metal workpiece is formed into a shaped (figure 5) or near-finally-shaped (figure 4) metal workpiece while the metal workpiece is in the second hardened condition. Figure 5 further specifies, in step 52, using a plurality of forming processes to form the shaped metal workpiece into a finally-shaped metal workpiece while in the second hardened condition. The method 50 includes performing 32 a first heat-treating process on a roughly-shaped metal workpiece in an annealed condition (with the workpiece in an annealed condition including at least one friction stir weld) to transition the roughly-shaped metal workpiece into a first hardened condition to produce a first-hardened metal workpiece. One example of the roughly-shaped metal workpiece is the metal workpiece 90 having at least one friction stir weld 92 as shown in figure 9, which is described in more detail below. The first hardened condition of the metal is the T4 condition when the metal workpiece is aluminum or an aluminum alloy.

The method 50 further includes performing 34 a second heat-treating process on the first-hardened metal workpiece to transition the first-hardened workpiece to a second hardened condition to produce a second-hardened metal workpiece. When the metal workpiece is aluminum or an aluminum alloy, the second hardened condition is the T6 condition.

The method 50 further includes forming 36 the second-hardened metal workpiece into a shaped metal workpiece, with the shaped metal workpiece being in one of a near-finally-shaped metal workpiece or a finally-shaped workpiece. An example of the shaped metal workpiece is the metal workpiece 114b, 114c, 114d, 114e, and 120 as shown in figures 11B, 11C, 11D, 11E, and figure 12, which is described in more detail below. According to aspects of the present disclosure, in method 50, forming processes 36 used to transform a roughly-shaped metal workpiece into the shaped (i.e., near-finally-shaped or finally-shaped) metal workpiece includes subjecting the metal workpiece to super-plastic processes, super-plastic/diffusion bond processes, form-die processes, explosive-forming processes, and combinations thereof. As contemplated by method 50, all of the forming processes on the roughly shaped metal workpiece (e.g., forming the roughly-shaped metal workpiece into the shaped metal workpiece) may be completed while the metal is in the second hardened condition.

The method 50 further includes using 52 a plurality of forming processes to form the shaped metal workpiece into the finally-shaped metal workpiece while the shaped metal workpiece is in the second hardened condition, with the forming processes set forth above for use in step 36 also contemplated as available forming methods in step 52. An example of the finally-shaped metal workpiece is the metal workpiece 114e and 120 as shown in figure 11E and figure 12, which is described in more detail below.

Consistent with particular aspects of the present disclosure, figure 6 is directed to a method 60 for making a heat-treated structure formed of metal. Method 60 is similar to method 50 outlined in figure 50, but includes forming 62 a metal sheet into a roughly-shaped metal workpiece including a friction stir weld, while the metal sheet is in the annealed condition. One example of the roughly-shaped metal workpiece is the metal workpiece 90 having at least one friction stir weld 92 as shown in figure 9, which is described in more detail below. The roughly-shaped state of the metal workpiece, according to aspects of the present disclosure, therefore contemplates the state of the metal work-piece between the initial form of a metal (e.g., a metal sheet that may be substantially planar) and a shaped (i.e., near-finally-shaped, or finally-shaped) metal workpiece that has been subjected to subsequent forming processes after attaining the roughly-shaped metal workpiece.

The method 60 further includes performing 32 a first heat-treating process on the roughly-shaped metal workpiece in an annealed condition (with the workpiece in an annealed condition comprising at least one friction stir weld) to transition the roughly-shaped metal workpiece into a first hardened condition to produce a first-hardened metal workpiece. The first hardened condition of the metal is the T4 condition when the metal workpiece is aluminum or an aluminum alloy.

The method 60 further includes performing 34 a second heat-treating process on the first-hardened metal workpiece to transition the first-hardened workpiece a second hardened condition to produce a second-hardened metal workpiece. When the metal workpiece is aluminum or an aluminum alloy, the second hardened condition is the T6 condition.

The method 60 further includes forming 36 the second-hardened metal workpiece into a shaped metal workpiece, with the shaped metal workpiece being in one of a near-finally-shaped metal workpiece or a finally-shaped workpiece. An example of the shaped metal workpiece is the metal workpiece 114b, 114c, 114d, 114e, and 120 as shown in figures 11B, 11C, 11D, 11E, and figure 12, which is described in more detail below. According to aspects of the present disclosure, the forming processes in the method 60 used to transform a roughly-shaped metal workpiece into the shaped (i.e., near-finally-shaped or finally-shaped) metal workpiece includes subjecting the metal sheet to super-plastic processes, super-plastic/diffusion bond processes, form-die processes, explosive-forming processes, and combinations thereof.

Method 60 further includes using 52 a plurality of forming processes to form the near-finally shaped metal workpiece into the finally-shaped metal workpiece while the near-finally-shaped metal workpiece is in the second hardened condition, with the forming processes set forth above for use in step 36 also contemplated as available forming methods in step 52. An example of the finally-shaped metal workpiece is the metal workpiece 114e and 120 as shown in figure 11E and figure 12, which is described in more detail below.

Consistent with particular aspects of the present disclosure, figure 7 is directed to a method 70 for making a heat-treated structure formed of metal. The method 70 described in figure 7 is similar to the method outlined in figure 1, except the method 70 contemplates 72 performing at least one age-hardening process on the roughly-shaped metal workpiece in the first hardened condition, and performing 74 at least one age-hardening process on the shaped metal workpiece in the second hardened condition. Method 70 therefore includes forming 12 a metal sheet into a roughly-shaped metal workpiece having a friction stir weld while the metal sheet is in an annealed condition. Step 12 is performed in a manner consistent with aspects of the present disclosure using forming processes including forming processes such as rolling or other physical shaping means suitable to physically transform and shape a metal from a first, or initial, orientation to a subsequent orientation. Further forming processes to transform metal to a roughly-shaped metal workpiece, as contemplated by aspects of the present disclosure, may take place in step 12 including subjecting the metal sheet to super-plastic processes, super-plastic/diffusion bond processes, form-die processes, explosive-forming processes, and combinations thereof. One example of the roughly-shaped metal workpiece is the metal workpiece 90 having at least one friction stir weld 92 as shown in figure 9, which is described in more detail below. The roughly-shaped state of the metal workpiece, according to aspects of the present disclosure, therefore contemplates the state of the metal workpiece between the initial form of a metal (e.g., a metal sheet that may be substantially planar) and a shaped (i.e., near-finally-shaped or finally-shaped) metal workpiece that has been subjected to subsequent forming processes after attaining the roughly-shaped metal workpiece.

Method 70 further includes performing 14 a first heat-treating process on the roughly-shaped metal workpiece to transition the roughly-shaped metal workpiece from an annealed condition comprising at least one friction stir weld to produce a first hardened condition, with the roughly-shaped metal workpiece comprising at least one friction stir weld. When the metal workpiece is aluminum or an aluminum alloy, the first hardened condition is the T4 condition.

The method 70 further includes performing 72 at least one age-hardening process on the roughly-shaped metal workpiece in the first hardened condition. When the metal workpiece is aluminum or an aluminum alloy and the first hardened condition is the T4 condition, the age-hardening process can be a natural aging process to age the metal workpiece to a stable condition.

The method 70 further includes forming 16 the roughly-shaped metal workpiece into a shaped metal workpiece while the roughly-shaped metal workpiece is in the first hardened condition. The shaped metal workpiece is one of a near-finally-shaped metal workpiece or a finally-shaped metal workpiece. An example of the shaped metal workpiece is the metal workpiece 114b, 114c, 114d, 114e, and 120 as shown in figures. 11B, 11C, 11D, 11E, and FIG 12, which is described in more detail below. According to aspects of the present disclosure, in step 16 the forming processes used to transform a roughly-shaped metal workpiece into the shaped (i.e., near-finally-shaped or finally-shaped) metal workpiece includes subjecting the metal sheet to super-plastic processes, super-plastic/diffusion bond processes, form-die processes, explosive-forming processes, and combinations thereof.

Method 70 further includes performing 18 a second heat-treating process on the shaped workpiece to transition the shaped metal workpiece from the first hardened condition to produce a second hardened condition. When the metal workpiece is aluminum or an aluminum alloy, the second hardened condition is the T6 condition.

The method 70 further includes performing 74 at least one age-hardening process on the shaped metal workpiece in the second-hardened hardened condition. When the metal workpiece is aluminum or an aluminum alloy and the second hardened condition is the T6 condition, the age-hardening process can be an artificial aging process to age the metal workpiece to achieve precipitation hardening.

At least one forming process can be performed while the metal is in the second hardened condition. However, all of the forming processes on the roughly-shaped workpiece (e.g., forming the roughly-shaped metal workpiece into the shaped metal workpiece) may be completed while the metal is in the first hardened condition.

Figures 8A, 8B, and 8C show a series in progression of exemplary drawings illustrating how a workpiece may be formed during an explosive forming process that can be used in the forming processes 16, 24, 36, 37, 42, and 52. According to explosive forming assembly 80a, a tank 82 contains an amount of water 83. A die 84 defines a cavity 85 and a vacuum line 87 extends from the cavity 85 through the die 84 to a vacuum (not shown). Workpiece 86a is held in position in the die 84 via a hold-down ring or other retaining device (not shown). An explosive charge 88 is shown suspended in the water 83 via a charge detonation line 89, with charge detonation line 19a connected to a detonator (not shown). As shown in figure 8B, the charge 88 (shown in figure 8A) has been detonated in explosive forming assembly 80b creating a shock wave "A" emanating from a gas bubble "B", with the shock wave "A" causing the deformation of the workpiece 86b into cavity 85 until the workpiece 86c is driven against (e.g., immediately proximate to and in contact with) the inner surface of die 84 as shown in figure 8C.

Consistent with particular aspects of the present disclosure, figure 9 is a perspective drawing of a metal workpiece 90 in an annealed condition and, for the purpose of the present disclosure, in a roughly-shaped condition or state. As shown in figure 9, workpiece 90 has been shaped into a substantially frusto-conical shape. Friction stir welds 92 are shown in workpiece 90, and are introduced into the metal workpiece before, after and/or during the forming of the metal workpiece into the roughly-shaped condition. While friction stir welds are shown, the present disclosure contemplates any welds that collectively can be referred to as "fly-away" welds as described herein. As shown, workpiece 90 is a metal workpiece that is preferably made from aluminum or an aluminum alloy or alloys. Workpiece 90 can be shaped into the frusto-conical orientation by forming processes, including forming processes such as rolling or other physical shaping means suitable to physically transform and shape a metal from a first, or initial, orientation (e.g., a metal sheet) to a subsequent roughly-shaped orientation, such as shown in figure 9.

Consistent with particular aspects of the present disclosure, figure 10 is a perspective view of a forming station 100. As shown in figure 10, workpiece 90 is introduced into forming block 102 that has a forming block cavity 104. The forming station 100 is nonspecific as to any particular forming process that can be used to shape metal workpieces. Representative forming processes include forming processes used to transform a roughly-shaped metal workpiece into the shaped (i.e., near-finally-shaped or finally-shaped) metal workpiece such as super-plastic processes, super-plastic/diffusion bond processes, form-die processes, explosive-forming processes (such as the process shown in figures 8A-8C), and combinations thereof, and include a forming block or die against which, by a force, a metal workpiece can be driven to achieve a predetermined shape.

Consistent with particular aspects of the present disclosure, figures 11A, 11B, 11C, 11D, and 11E are cross-sectional side views showing a section of a workpiece within forming blocks, and showing the progressive forming and shaping of a workpiece from a roughly-shaped workpiece 90 as shown in figures 9 and 10 into a near-finally and/or finally-shaped workpiece.

Figure 11A shows a cross-sectional side view of forming block 102 taken across line "A" of forming block 102 as shown in figure 10. figure 11A, in step 110a, shows cross-section of roughly-shaped metal workpiece 90 resting within the cavity of forming block 112a (a cross-section of forming block 102 taken along line "A" as shown in figure 10). After workpiece 90 has been exposed to at least one forming process, figure 11B shows step 110b, wherein roughly-shaped metal workpiece 90 is now shown as 114b having been shaped such that the roughly-shaped metal workpiece rests substantially proximate to the wall 113a of cavity 115. The roughly-shaped workpiece 90 is thus transformed into shaped workpiece 114b. Shaped workpiece 114c is shown as having been further shaped as compared to the shaped workpiece 114b shown in figure 11B.

As shown in figure 11C, shaped workpiece 114b has been further shaped into workpiece 114c by trimming workpiece end 114c' of workpiece 114c. Figure 11D shows a second forming block 112b having a wall 113b with a contour that is different from the contour of wall 113a of forming block 112a. The wall 113b defines a cavity of the second forming block 112b. In this way, forming block 112b has a different cavity configuration as compared to the cavity of forming block 112a. As shown in step 110c, the workpiece 114c has now been subjected to a further forming process and further shaped into a workpiece configuration shown as workpiece 114d. Figure 11E shows step 110e wherein workpiece 114d has been further shaped by a further forming process followed by a trimming operation to shape workpiece end 114e' of workpiece 114e. According to aspects of the present disclosure, workpieces 90, 114b, and 114c can be considered to be a roughly-shaped workpiece, while workpieces 114d and 114e are shown to be a nearly-finally shaped workpiece. In further aspects, workpieces 114d and/or 114e may be considered to be finally-shaped workpieces, depending upon the desired and predetermined configuration of the workpiece according to the final workpiece configuration needed in use. According to further aspects (not shown) additional forming steps may be used, requiring additional forming blocks, if desired.

Figure 12 is a perspective view of a nacelle lipskin according to an aspect of the present disclosure. As shown in figure 12, a lipskin 120 is fabricated according to methods disclosed herein, and ready for installation to an aircraft engine nacelle 132 on an aircraft 130 as shown in figure 13.

According to aspects of the present disclosure, the forming processes are conducted while the metal workpiece is in the first hardened condition. The present disclosure further contemplates aspects where some of the forming processes may be conducted while the metal workpiece is in the second hardened condition. However, such forming of the workpiece in the second hardened condition will be finished forming and shaping; in some cases modifying the metal workpiece less than about 3% of the forming conducted on the metal workpiece as compared with the forming conducted on the workpiece when the workpiece is in conditions other than the second hardened condition. The present disclosure therefore contemplates forming the metal workpiece via forming processes conducted: 1) in the annealed and first hardened conditions; 2) in the annealed and in either the first hardened or second hardened conditions; and 3) in the annealed and both the first hardened and second hardened conditions.

According to aspects of the present disclosure, friction stir welds that are incurred in the metal workpieces produced according to the methods presented herein are retained in the near-finally-shaped and/or finally-shaped metal workpieces. In other words, the friction stir weld(s) made in the metal workpieces are not removed in finishing steps. As a result, the need for couplers or other reinforcing component parts (e.g. rivets, fasteners, etc.) is obviated according to aspects of the present disclosure.

Aspects of the present disclosure may, of course, be carried out in other ways than those specifically set forth herein without departing from essential characteristics of the aspects presented herein.

## Claims

1. A method for making a heat-treated structure formed of metal, such as an engine nacelle for an aircraft, the method comprising:
performing a first heat-treating process on a roughly-shaped metal workpiece in an annealed condition to transition the roughly-shaped metal workpiece from the annealed condition into a first hardened condition, the roughly-shaped metal workpiece in the annealed condition comprising at least one friction stir weld;
forming the roughly-shaped metal workpiece into a shaped metal workpiece while the roughly-shaped metal workpiece is in the first hardened condition, the shaped metal workpiece comprising one of a near-finally-shaped metal workpiece or a finally-shaped metal workpiece; and
performing a second heat-treating process on the shaped metal workpiece to transition the shaped metal workpiece from the first hardened condition to a second hardened condition,
wherein the forming process is selected from the group consisting of: a super-plastic forming process; a super-plastic/diffusion bond forming process; an explosion forming process; and combinations thereof,
wherein performing the first heat-treating process comprises performing a T4 heat-treating process on the roughly-shaped metal workpiece,
wherein the metal is a 2000-, 4000-, 6000-, or 7000-series aluminum alloy.

2. The method according to claim 1, comprising forming the second hardened metal workpiece into a shaped metal workpiece, said shaped metal workpiece being one of a near-finally-shaped metal workpiece or a finally-shaped metal workpiece.

3. The method according to claim 2, wherein the shaped metal workpiece is, or comprises, a near-finally-shaped metal workpiece, the method further comprising:
forming the near-finally-shaped metal workpiece into the finally-shaped metal workpiece while the near-finally-shaped metal workpiece is in the second hardened condition.

4. The method according to claim 2 or 3, wherein the shaped metal workpiece comprises a finally-shaped metal workpiece, the method further comprising using one or more forming processes to shape the roughly-shaped metal workpiece into the finally-shaped metal workpiece.

5. The method according to any of the preceding claims, wherein, before the step of performing the first heat-treating process on the roughly-shaped metal workpiece, a metal sheet is formed into the roughly-shaped metal workpiece while the metal sheet is in the annealed condition, preferably wherein the step of forming a metal sheet comprises rolling the metal sheet into the roughly-shaped metal workpiece.

6. The method according to claim 5, wherein the metal sheet is in an annealed condition, and is formed into the roughly-shaped metal workpiece by a process selected from the group consisting of: a super-plastic forming process; a super-plastic/diffusion bond forming process; a form-die forming process; an explosion forming process; and combinations thereof.

7. The method according to any of the preceding claims, wherein the roughly-shaped workpiece is a conical-shaped metal workpiece or a frusto-conical-shaped metal workpiece.

8. The method according to any of the preceding claims, wherein the step of performing the second heat-treating process further comprises:
performing at least one age-hardening process on the roughly-shaped metal workpiece in the first and/or second hardened condition.

9. The method according to claim 8, wherein the age-hardening process is a natural aging process when the roughly-shaped metal is in the first hardened condition and wherein the age-hardening process is an artificial aging process when the roughly shaped metal is in the second hardened condition.

10. The method according to any of the preceding claims, wherein the second hardened condition comprises a second age-hardened condition.

11. The method according to any of the preceding claims, wherein the step of performing the second heat-treating process further comprises solution heat-treating the metal.

12. The method according any one of the preceding claims, wherein performing the second heat-treating process comprises performing a T6 heat-treating process.

## Patentansprüche

1. Verfahren zum Herstellen einer wärmebehandelten Struktur aus Metall, wie etwa einer Triebwerksgondel für ein Flugzeug, wobei das Verfahren Folgendes umfasst:
Durchführen eines ersten Wärmebehandlungsprozesses an einem grob geformten Metallwerkstück in einem geglühten Zustand, um das grob geformte Metallwerkstück von dem geglühten Zustand in einen ersten gehärteten Zustand zu überführen, wobei das grob geformte Metallwerkstück in dem geglühten Zustand mindestens eine Reibrührschweißnaht umfasst;
Umformen des grob geformten Metallwerkstücks in ein geformtes Metallwerkstück, während sich das grob geformte Metallwerkstück in dem ersten gehärteten Zustand befindet, wobei das geformte Metallwerkstück ein nahezu fertig geformtes Metallwerkstück oder ein endgültig geformtes Metallwerkstück umfasst; und
Durchführen eines zweiten Wärmebehandlungsprozesses an dem geformten Metallwerkstück, um das geformte Metallwerkstück von dem ersten gehärteten Zustand in einen zweiten gehärteten Zustand zu überführen,
wobei der Formgebungsprozess aus der Gruppe ausgewählt ist, die aus Folgendem besteht: einem superplastischen Formgebungsprozess; einem superplastischen/Diffusionsbindungsformprozess; einem Explosionsformprozess; und Kombinationen davon,
wobei das Durchführen des ersten Wärmebehandlungsprozesses das Durchführen eines T4-Wärmebehandlungsprozesses an dem grob geformten Metallwerkstück umfasst,
wobei es sich bei dem Metall um eine Aluminiumlegierung der 2000er-, 4000er-, 6000er- oder 7000er-Serie handelt.

2. Verfahren nach Anspruch 1, umfassend das Umformen des zweiten gehärteten Metallwerkstücks zu einem geformten Metallwerkstück, wobei das geformte Metallwerkstück ein nahezu fertig geformtes Metallwerkstück oder ein endgültig geformtes Metallwerkstück ist.

3. Verfahren nach Anspruch 2, wobei das geformte Metallwerkstück ein nahezu fertig geformtes Metallwerkstück ist oder umfasst, wobei das Verfahren ferner Folgendes umfasst:
Umformen des nahezu fertig geformten Metallwerkstücks in das fertig geformte Metallwerkstück, während sich das nahezu fertig geformte Metallwerkstück in dem zweiten gehärteten Zustand befindet.

4. Verfahren nach Anspruch 2 oder 3, wobei das geformte Metallwerkstück ein endgültig geformtes Metallwerkstück umfasst, wobei das Verfahren ferner das Verwenden eines oder mehrerer Umformprozesse umfasst, um das grob geformte Metallwerkstück in das endgültig geformte Metallwerkstück zu formen.

5. Verfahren nach einem der vorhergehenden Ansprüche, wobei vor dem Schritt des Durchführens des ersten Wärmebehandlungsprozesses an dem grob geformten Metallwerkstück ein Metallblech zu dem grob geformten Metallwerkstück geformt wird, während sich das Metallblech im geglühten Zustand befindet, wobei der Schritt des Umformens eines Metallblechs vorzugsweise das Walzen des Metallblechs zu dem grob geformten Metallwerkstück umfasst.

6. Verfahren nach Anspruch 5, wobei sich das Metallblech in einem geglühten Zustand befindet und zu dem grob geformten Metallwerkstück umgeformt wird durch einen Prozess, der aus der Gruppe ausgewählt ist, die aus Folgendem besteht: einem superplastischen Formungsprozess; einem superplastischen/Diffusionsbindungsformprozess; einem Formmatrizenformprozess; einem Explosionsformprozess; und Kombinationen davon.

7. Verfahren nach einem der vorhergehenden Ansprüche, wobei es sich bei dem grob geformten Werkstück um ein konisch geformtes Metallwerkstück oder ein kegelstumpfförmiges Metallwerkstück handelt.

8. Verfahren nach einem der vorhergehenden Ansprüche, wobei der Schritt des Durchführens des zweiten Wärmebehandlungsprozesses ferner Folgendes umfasst:
Durchführen mindestens eines Aushärtungsprozesses an dem grob geformten Metallwerkstück in dem ersten und/oder zweiten gehärteten Zustand.

9. Verfahren nach Anspruch 8, wobei es sich bei dem Aushärtungsprozess um einen natürlichen Alterungsprozess handelt, wenn sich das grob geformte Metall in dem ersten gehärteten Zustand befindet, und wobei es sich bei dem Aushärtungsprozess um einen künstlichen Alterungsprozess handelt, wenn sich das grob geformte Metall in dem zweiten gehärteten Zustand befindet

10. Verfahren nach einem der vorhergehenden Ansprüche, wobei der zweite gehärtete Zustand einen zweiten ausgehärteten Zustand umfasst.

11. Verfahren nach einem der vorhergehenden Ansprüche, wobei der Schritt des Durchführens des zweiten Wärmebehandlungsprozesses ferner ein Lösungsglühen des Metalls umfasst.

12. Verfahren nach einem der vorhergehenden Ansprüche, wobei das Durchführen des zweiten Wärmebehandlungsprozesses das Durchführen eines T-6 Wärmebehandlungsprozesses umfasst.

## Revendications

1. Procédé de production d'une structure thermotraitée en métal, telle qu'un fuseau moteur d'aéronef, le procédé comprenant :
la réalisation d'un premier processus de traitement thermique sur une pièce ouvrée en métal grossièrement mise en forme à l'état recuit afin de faire passer la pièce ouvrée en métal grossièrement mise en forme de l'état recuit à un premier état trempé, ladite pièce ouvrée en métal grossièrement mise en forme à l'état recuit comprenant au moins une soudure par friction-malaxage,
le formage de la pièce ouvrée en métal grossièrement mise en forme en une pièce ouvrée en métal mise en forme pendant que la pièce ouvrée en métal grossièrement mise en forme se trouve audit premier état trempé, ladite pièce ouvrée en métal mise en forme comprenant une pièce ouvrée en métal mise en forme quasi finale ou une pièce ouvrée en métal mise en forme finale, et
la réalisation d'un deuxième processus de traitement thermique sur la pièce ouvrée en métal mise en forme afin de faire passer la pièce ouvrée en métal mise en forme du premier état trempé à un deuxième état trempé ;
ledit processus de formage appartenant au groupe constitué par : un processus de formage superplastique, un processus de formage superplastique et d'assemblage par diffusion, un processus de formage par explosion, et des combinaisons de ceux-ci,
ladite réalisation du premier processus de traitement thermique comprenant la réalisation d'un processus de traitement thermique T4 sur la pièce ouvrée en métal grossièrement mise en forme,
ledit métal étant un alliage d'aluminium de la série 2000, 4000, 6000 ou 7000.

2. Procédé selon la revendication 1, comprenant le formage de la deuxième pièce ouvrée en métal trempé en une pièce ouvrée en métal mise en forme, ladite pièce ouvrée en métal mise en forme étant une pièce ouvrée en métal mise en forme quasi finale ou une pièce ouvrée en métal mise en forme finale.

3. Procédé selon la revendication 2, dans lequel la pièce ouvrée en métal mise en forme est ou comprend une pièce ouvrée en métal mise en forme quasi finale, le procédé comprenant en outre :
le formage de la pièce ouvrée en métal mise en forme quasi finale en la pièce ouvrée en métal mise en forme finale pendant que la pièce ouvrée en métal mise en forme quasi finale se trouve dans ledit deuxième état trempé.

4. Procédé selon la revendication 2 ou 3, dans lequel la pièce ouvrée en métal mise en forme comprend une pièce ouvrée en métal mise en forme finale, le procédé comprenant en outre la mise en oeuvre d'un ou plusieurs processus de formage afin de mettre en forme la pièce ouvrée en métal grossièrement mise en forme en ladite pièce ouvrée en métal mise en forme finale.

5. Procédé selon l'une quelconque des revendications précédentes, dans lequel, avant l'étape de réalisation du premier processus de traitement thermique sur la pièce ouvrée en métal grossièrement mise en forme, une tôle de métal est façonnée en la pièce ouvrée en métal grossièrement mise en forme pendant que la tôle de métal se trouve à l'état recuit, l'étape de formage de la tôle de métal comprenant de préférence le laminage de la tôle de métal en ladite pièce ouvrée en métal grossièrement mise en forme.

6. Procédé selon la revendication 5, dans lequel la tôle de métal se trouve à l'état recuit et est façonnée en ladite pièce ouvrée en métal grossièrement mise en forme selon un processus appartenant au groupe constitué par : un processus de formage superplastique, un processus de formage superplastique et d'assemblage par diffusion, un processus de formage par matrice de formage, un processus de formage par explosion, et des combinaisons de ceux-ci.

7. Procédé selon l'une quelconque des revendications précédentes, dans lequel la pièce ouvrée grossièrement mise en forme est une pièce ouvrée en métal de forme conique ou une pièce ouvrée en métal de forme frustoconique.

8. Procédé selon l'une quelconque des revendications précédentes, dans lequel l'étape de réalisation du deuxième processus de traitement thermique comprend en outre :
la réalisation d'au moins un processus de durcissement par vieillissement sur la pièce ouvrée en métal grossièrement mise en forme se trouvant au premier et/ou au deuxième état trempé.

9. Procédé selon la revendication 8, dans lequel le processus de durcissement par vieillissement est un processus de vieillissement naturel lorsque le métal grossièrement mis en forme se trouve dans ledit premier état trempé et dans lequel le durcissement par vieillissement est un processus de vieillissement artificiel lorsque le métal grossièrement mis en forme se trouve dans ledit deuxième état trempé.

10. Procédé selon l'une quelconque des revendications précédentes, dans lequel le deuxième état trempé comprend un deuxième état de durcissement par vieillissement.

11. Procédé selon l'une quelconque des revendications précédentes, dans lequel l'étape de réalisation du deuxième processus de traitement thermique comprend en outre le traitement thermique du métal par mise en solution.

12. Procédé selon l'une quelconque des revendications précédentes, dans lequel la réalisation du deuxième processus de traitement thermique comprend la réalisation d'un processus de traitement thermique T6.
